

## UNITED STATES PATENT OFFICE.

GEORGE C. HANNAM, OF FREEPORT, AND JULIUS W. SCHEDE, OF MOUNT VERNON, NEW YORK, ASSIGNEES TO RUBBERSTONE CORPORATION, OF NEW YORK, N. Y., A CORPORATION OF NEW YORK.

## FLOORING TILE.

No Drawing.

Application filed January 31, 1927. Serial No. 185,028.

Our invention relates to flooring tile and while we use this term "flooring tile" to designate one use of the tile it is of course to be understood that the tile may be used 5 on walls or other surfaces and that we do not wish to be limited by the term employed.

An object of the invention is to provide a tile that will be free from pot marks, which will have a hard surface, that can be easily 10 washed and that will not allow the dirt to be readily ground into the surface and which will hold its original color.

A further object is to provide a tile that will have the maximum of tensile strength 15 and flexibility so as to minimize breaking or cracking and which will have the maximum of wearing qualities.

A further object is to provide a tile of 20 novel composition which can be given a desired color and which will retain the color in use.

With these and other objects in view, the invention consists in certain novel combinations of ingredients which will now be 25 described and hereinafter pointed out in the claim.

Our improved composition comprises pitch, gum, fiber and a coloring matter.

We preferably employ a pitch which will 30 break down brown and find that vegetable pitch will give this result.

Specifically stated, the composition is as follows:

|                                     | Pounds.         |
|-------------------------------------|-----------------|
| 35 Vegetable pitch                  | $18\frac{1}{3}$ |
| "Cumar" gum (a coal tar derivative) | $3\frac{2}{3}$  |
| Asbestos fiber                      | 40              |
| Coloring matter.                    |                 |

These ingredients are mixed in any suitable apparatus under a temperature of approximately four hundred degrees Fahrenheit, and we of course do not limit ourselves to the particular manner of mixing but we find in ordinary practice the pitch and the gum may first be mixed and the fiber then added.

The coloring matter may be added at any time and may be of many different materials in accordance with the color desired, and the proportions of the coloring matter will of course vary.

While we have set forth what we believe to be a preferred composition, it is to be understood that the invention is capable of modification in the arrangement and proportions of the ingredients, and we do not wish to be limited to the specific formula set forth but desire to cover the invention as set forth in the claim.

## We claim:

A tile composition, comprising vegetable pitch, light "Cumar" gum (a coal tar derivative), and asbestos fiber in substantially the proportions of pitch thirteen and a third pounds, light "Cumar" gum three and two-thirds pounds, and asbestos fiber forty pounds.

GEORGE C. HANNAM.  
JULIUS W. SCHEDE.